

Dec. 20, 1927.

1,653,592

J. W. STRATMAN

WINDOW SHADE CLOTH AND PROCESS OF CONSTITUTING

Filed Feb. 27, 1926



Inventor

*Joseph W. Stratman*

By

*Wood-Wood*

Attorneys

## UNITED STATES PATENT OFFICE.

JOSEPH W. STRATMAN, OF CINCINNATI, OHIO, ASSIGNOR TO THE CHAS. W. BRENEMAN COMPANY, OF CINCINNATI, OHIO, A CORPORATION OF OHIO.

## WINDOW-SHADE CLOTH AND PROCESS OF CONSTITUTING.

Application filed February 27, 1926. Serial No. 91,277.

My invention relates to window shade cloth, and to a process for making the same.

My invention particularly is directed to a window shade cloth combining certain physical properties and advantages with desirable ornamental or decorative effects. My invention also includes the preferred process of manufacturing the window shade cloth having said advantages and effects.

10 The object of my invention is to provide a light flexible window shade cloth which will not crack or fade, which is not injured by exposure to moisture, and which will have a permanent and decorative structure.

15 Another object of my invention is to provide a configurated ornamental window shade cloth which is adapted to roll readily on the conventional window shade roller.

20 Another object of my invention is to provide a process of manufacturing such a window shade cloth.

25 Another object of my invention is to provide an economical process of constituting and manufacturing a durable and ornamental window shade cloth.

30 Other objects and certain advantages will be more fully set forth in the description of the accompanying drawings forming a part of this specification, in which:

The figure of the drawing illustrates a length of window shade cloth stretched on the processing frame.

35 For purposes of illustration, the window shade cloth is disclosed as bearing a striped ornamentation.

The stretching frame comprises an upper member 1 which is suspended as by chains 2. The cloth 3 is stretched between 40 this upper member 1 and a lower member 4, the cloth being glued or otherwise attached to each member. Stretching pieces 5 are hinged to the lower member 4 by means of bolts 6 passing through both. These frame

45 members and stretching pieces may be ordinary wooden two by fours. The upper member is provided with sockets 7 each one directly above a hinge between a stretching piece and the lower member. These sockets

50 are open at one side in order that the stretching members may be swung into the sockets and are secured to the top frame member by bolts 8. The portions of the stretching members adapted to enter the

55 sockets are provided with lineally extending

rows of apertures 9. The faces of the sockets are provided with apertures 10 aligned with the rows of apertures 8 when the stretching members are seated in the sockets. Pins 11 are attached to the upper frame member by means of chains 13. These pins are adapted to enter the socket and stretching member apertures in order to hold the upper and lower frame members the desired distance apart and stretch the cloth between 65 to the proper extent.

In constituting and manufacturing the window shade cloth, a length of the cloth itself is secured on the frame. The ornamentation is constituted by the weave of the 70 cloth. One cloth suitable for the disclosed purposes, is a muslin weighing approximately 123½ grams per square yard. As disclosed, the ornamental configuration consists of stripe which is in the weave of the 75 muslin, the threads being closer together over the striped portions, thereby defining them visually and physically.

The cloth is then stretched on the frame and allowed to dry. Great care must be 80 taken to stretch such a cloth on the frame with the stripes perfectly straight.

Due to the relatively heavy texture of the striped portions of the cloth, it is necessary 85 to convert it into the finished window shade cloth without increasing too greatly its weight. Moreover, the heavier portions of the cloth give the same a certain body which permits the cloth to roll properly on the shade roller without the conventional 90 relatively heavy finishing coatings.

The cloth is next sized with water solution of a high quality of hide glue having zinc oxide suspended therein. The best quality and most finely ground zinc oxide 95 obtainable is recommended in order that it be dispersed as thickly and evenly as possible throughout the glue. The solution is formed by dissolving one pound of the zinc oxide containing glue in between thirty-five and forty pounds of water. This solution is approximately one-half as concentrated as the conventional sizing solution.

This is a material saving financially. The sizing is applied with brushes or in 105 any conventional manner.

The next step is to paint the sized cloth with oil paints. For this configurated muslin shade cloth, paints containing only coloring compounds chemically pure such as lead 110

chromates, sienna, sublimed lead, lithopone umber, ochre and ultramarine blue are recommended. The paint is thinned down to about 15° Bé. (light liquid scale) with 5 naphtha and benzine and the sized cloth painted therewith on both sides. This paint is materially lighter than the standard window shade cloth paints which range in weight between 35° and 10° Bé. (heavy 10 liquid scale).

The paint is allowed to dry after which the window shade cloth is removed from the stretching frames and cut to the desired dimensions.

15 Thus I provide a durable ornamental configurated window shade cloth relatively economical to manufacture and of proper weight and flexibility to be used on the conventional window shade rollers.

Having described my invention, I desire 29 to be limited only by the following claim:

The process of making ornamental window shade cloth comprising the steps of 25 sizing a length of muslin, having stripes woven therein, said muslin weighing approximately 123½ grams per square yard, with a glue containing zinc oxide, said glue diluted with water in the proportion of one pound of glue to between thirty-five and forty pounds of water, and painting the 30 sized surfaces with oil paints of approximately 15° Bé. (light liquid scale) in order to form a window shade cloth of proper weight and flexibility to roll upon a window shade roller.

In witness whereof, I hereunto subscribe my name.

JOSEPH W. STRATMAN.